# EUROPEAN PATENT SPECIFICATION

(11) **EP 2 808 411 B1**
(45) Date of publication and mention of the grant of the patent: **23.08.2017**
(21) Application number: 12866465.3
(22) Date of filing: 25.04.2012
(51) Int. Cl.: C21D 6/00, C22C 38/02, C22C 38/04, C22C 38/06, C22C 38/08, C22C 38/16, C22C 38/18, C22C 38/40, C22C 38/42, C22C 38/00, C22C 38/60

(54) **CORROSION-RESISTANT STEEL FOR HOLD OF COAL CARRYING VESSEL OR COAL/ORE CARRYING VESSEL**
KORROSIONSBESTÄNDIGER STAHL ZUM HALTEN EINES KOHLEGEFÄSS ODER EINES KOHLE/ERZ-GEFÄSSES
ACIER RÉSISTANT À LA CORROSION DESTINÉ À LA CALE D'UN TRANSPORTEUR DE CHARBON OU D'UN TRANSPORTEUR DE CHARBON/MINERAI

(30) Priority: 25.01.2012 JP 2012012530
(43) Date of publication of application: 03.12.2014
(73) Proprietor: JFE Steel Corporation, Tokyo 100-0011 (JP)
(72) Inventor: OMODA, Masataka, Tokyo 100-0011 (JP); TSURI, Shiro, Tokyo 100-0011 (JP); KOMORI, Tsutomu, Tokyo 100-0011 (JP); HOSHINO, Toshiyuki, Tokyo 100-0011 (JP)
(74) Representative: Hoffmann Eitle
(86) International application number: PCT/JP2012/061624
(87) International publication number: WO 2013/111355

(56) References cited:
- EP-A1- 1 460 145
- EP-A1- 1 990 437
- JP-A- H0 953 149
- JP-A- H0 971 837
- JP-A- 2000 017 382
- JP-A- 2003 213 367
- JP-A- 2007 262 558
- YUKI KOBAYASHI ET AL.: 'Corrosion and Corrosion Fatigue of a Ship Structural Steel in Dilute Sulfuric Acids Substituted for a Corrosion Environment of a Coal Cargo Hold' JOURNAL OF THE SOCIETY OF NAVAL ARCHITECTS OF JAPAN June 1999, pages 221 - 232, XP055081739
- AKIRA USAMI ET AL.: 'New S-TEN1: an Innovative Acid Resistant Low Alloy Steel' SHINNITTETSU GIHO no. 380, 15 June 2004, pages 86 - 90, XP055136765
- D.P. LE ET AL.: 'Effect of antimony on the corrosion behavior of low-alloy steel for flue gas desulfurization system' CORROSION SCIENCE vol. 50, no. 4, April 2008, pages 1195 - 1204, XP003031083

## Description

### [Technical Field]

The present invention relates to a steel with excellent corrosion resistance used for a coal carrier or ore/coal carrier hold (may be referred to as belly of a ship).

### [Background Art]

At the beginning of the 1990s, successive maritime accidents of bulk carriers caused international problems. In particular, many accidents of coal carriers and ore/coal carriers were reported and most of causes thereof were damages in bellies of ships. In the bulk carrier, a cargo is loaded directly in a hold and, therefore, an influence of a corrosive cargo is exerted easily. It is believed to be a problem that the strength is reduced locally by corrosion in a belly of a ship (hereafter may be referred to as "hold"), in particular, pitting corrosion of a side shell in a hold of a coal carrier or ore/coal carrier. Instances in which this pitting corrosion proceeded significantly and instances in which the plate thickness of a side frame portion to ensure the strength of a carrier was reduced considerably have been reported. In order to prevent an accident, Non Patent Literature 1 stipulates that renewal of a hold side shell steel is required in the case of 70% or less of the as-built thickness and renewal of a hold side frame steel is required in the case of 75% or less of the as-built thickness (where a value larger than the as-built thickness - corrosion allowance - voluntary thickness addition is not required).

The side shell of a bulk carrier in which the above-described pitting corrosion occurs is a single-hull, and a cargo and the seawater is separated by only a plate of steel. Then, the temperature in the hold increases on the basis of self-heating inherent in the coal. Consequently, dew condensation water is generated easily on the hold side shell because of a temperature difference between the seawater and the inside of the hold. The inside of the hold is in a low pH environment in which sulfuric acid corrosion occurs easily because SO₄²⁻ in the coal is eluted into the above-described place where dew condensation water has been generated on the hold side shell and reacts with the dew condensation water to generate sulfuric acid. Therefore, two corrosion protection mechanisms are required, where "inhibition of hydrogen generation reaction" is performed against the low pH environment and "inhibition of SO₄²⁻ permeation in rust layers" is performed against SO₄²⁻ permeation to rust/steel interface, while SO₄²⁻ serves as a counter anion to dissolution of iron.

Modified epoxy resin coating having a coating thickness of about 150 to 200 µm is applied to the inside of the hold as the above-described corrosion control method in the hold. However, in many cases, the coatings are peeled because of mechanical damages by coals and iron ores and flaws abrasions due to heavy machinery in cargo carrying out, so that a sufficient effect of corrosion protection is not obtained.

Then, periodic repainting and partial touch-up methods have been employed as further corrosion control methods. However, such methods require very large costs. Therefore, reduction in the life cycle cost including the maintenance cost of ship remains an issue.

Meanwhile, as for corrosion-resistant steels for ships, steels developed for cargo oil tanks and ballast tanks have been known.

An upper deck of cargo oil tank side is exposed to an environment of corrosive gases, e.g., O₂, CO₂, and SO₂ contained in an inert gas blown into a tank for the purpose of explosion protection and H₂S and the like volatilized from crude oil. Although a bottom plate has a protective film (may be referred to as "oil coat") derived from crude oil, a place where the film has been peeled is exposed to an environment in which bowl-shaped local corrosion occurs. For example, Patent Literature 1 proposes a corrosion-resistant steel by utilizing corrosion protection mechanisms for "improvement in corrosion resistance on the basis of inhibition of pH reduction" and "improvement in local corrosion resistance on the basis of sulfide fine dispersion".

Also, when no cargo is loaded, the ballast tank is poured with the seawater to perform a function of allowing a ship to achieve stable navigation and, therefore, is placed in a very severe corrosive environment. The upper deck of ballast tank side is not immersed into the seawater, nor is in the state of being sprayed with the seawater. Consequently, cathodic protection does not function and, in addition, this area comes into a severe corrosive environment because the temperature of the steel increases by sunshine, and undergoes severe corrosion. Meanwhile, the side shell surface and the bottom of the ballast tank are portions immersed in the seawater completely and are in a corrosive environment, although a cathodic protection action functions.

However, in the navigation with cargo, the seawater is not poured into the ballast tank, and the cathodic protection does not function at all with respect to the whole ballast tank. Therefore, severe corrosion occurs because of a cyclic wet and dry environment and actions of residual adhesion salts. For example, Patent Literature 2 proposes that Cl⁻ permeation is inhibited by densification of rust and Patent Literature 3 proposes a corrosion-resistant steel by utilizing a corrosion protection mechanism in which Cl⁻ permeation is electrochemically inhibited by WO₄²⁻.

As described above, in the coal carrier or ore/coal carrier, it is necessary that a hydrogen generation reaction be inhibited and SO₄²⁻ permeation to rust/steel interface be inhibited in the case of low pH environment in which concentration of sulfuric acid occurs because of the cyclic wet and dry environment. As described above, the corrosive environments and the corrosion protection mechanisms are different between the coal carrier or ore/coal carrier holds, ballast tanks, and the oil tanks and, therefore, the corrosion-resistant steels for the ballast tank or the oil tank cannot be diverted on an "as is" basis. Consequently, as for the steel for the coal carrier or ore/coal carrier hold, original material design and characteristic evaluation are required.

Also, Patent Literatures 1, 4, and 5 are mentioned as the related art referring to the coal carrier or ore/coal carrier hold use. As for the chemical compositions of corrosion-resistant steels for shipbuilding in the use environment of the coal carrier or ore/coal carrier hold, Patent Literature 1 discloses a steel containing Cu and Mg as indispensable chemical compositions, Patent Literature 4 discloses a steel containing Cu, Ni, and Sn as indispensable chemical compositions, and Patent Literature 5 discloses a steel containing Cu and Sn as indispensable chemical compositions for the purpose of further improving the cost.

Patent Literature 6 (PTL 6) relates to a corrosion-resistant steel material for ship and vessel containing, in mass percent, C of 0.03 to 0.25%, Si of 0.05 to 0.50%, Mn of 0.1 to 2.0%, P of 0.025% or less, S of 0.01% or less, Al of 0.005 to 0.10%, W of 0.01 to 1.0%, Cr of 0.01% or more and less than 0.20%, and furthermore containing as needed one or two selected from Sb of 0.001 to 0.3% and Sn of 0.001 to 0.3% and/or one or at least two selected from Ni of 0.005 to 0.25%, Mo of 0.01 to 0.5% and Co of 0.01 to 1.0%, and containing the remainder including Fe and inevitable impurities.

Patent Literature 7 (PTL 7) discloses a low alloy steel and weld joint thereof containing, in mass, C of 0.001 to 0.2%, Si of 0.01 to 2.5%, Mn of 0.1 to 2%, Cu of 0.1 to 1%, Mo of 0.001 to 1%, Sb of 0.01 to 0.2%, P of 0.05% or less and S of 0.05% or less with the balance consisting of Fe and unavoidable impurities.

### [Citation List]

### [Non Patent Literature]

[NPL 1] Nippon Kaiji Kyokai, COMMON STRUCTURAL RULES FOR BULK CARRIERS (RULES FOR THE SURVEY AND CONSTRUCTION OF STEEL SHIPS PART CSR-B), p. 384-394, (2006)

### [Patent Literature]

[PTL 1] Japanese Unexamined Patent Application Publication No. 2000-17381
[PTL 2] Japanese Unexamined Patent Application Publication No. 2008-144204
[PTL 3] Japanese Unexamined Patent Application Publication No. 2007-46148
[PTL 4] Japanese Unexamined Patent Application Publication No. 2007-262555
[PTL 5] Japanese Unexamined Patent Application Publication No. 2008-174768
[PTL 6] European Patent Application Publication EP 1 990 437 A1
[PTL 7] European Patent Application Publication EP 1 460 145 A1

### [Summary of Invention]

### [Technical Problem]

However, the subject of the steel shown in Patent Literature 1 is a steel excellent in the use environment common to ship shells, ballast tanks, cargo oil tanks, ore carrier cargo holds, and the like. Therefore, good results in the corrosion test of the cargo oil tank and the ballast tank are mentioned as the method for evaluating the corrosion resistance of the steel, although test results in consideration of the use environments of the coal carrier and ore/coal carrier holds are not shown.

Also, in Patent Literatures 4 and 5, the corrosion resistance under coating film is evaluated, where an environment of the coal carrier or ore/coal carrier hold is simulated. However, an evaluation test simulating the case where peeling occurs easily because of mechanical damages by coals and iron ores, which can be said to be unavoidable in the use environment of the hold, and an evaluation of maximum pitting corrosion depth serving as a renewal guideline of the steel plate are not performed.

As described above, consideration of corrosion environment specific to the coal carrier or ore/coal carrier hold and, in addition, an evaluation of corrosion of a steel in the state of having no coating film because of peeing of the coating film are important for the development of a steel with excellent corrosion resistance to be used for the coal carrier or ore/coal carrier hold. However, these viewpoints are not taken into consideration in the related art.

Accordingly, it is an object of the present invention to provide a corrosion-resistant steel according to claim 1 for a coal carrier or ore/coal carrier hold, wherein corrosion after peeling of a coating film can be inhibited under a cyclic wet and dry environment and a low pH environment.

### [Solution to Problem]

In general, a ship is built by welding steels, e.g., steel plates, steel sheets, shaped steels, and steel bars, and corrosion protection coating films are applied to the surfaces of the steels to be used. However, in the environment of the coal carrier or ore/coal carrier hold, the coating is in the circumstances of being peeled easily because of mechanical damages by coals and ores, and the steel is exposed to a cyclic wet and dry environment and a low pH environment. Here, a steel capable of exerting the corrosion resistance even after peeling of a surface corrosion protection coating film of the steel has been developed.

In this regard, the present inventors developed a testing method simulating an environment in a coal carrier or ore/coal carrier hold, and studied influences of the individual alloy elements by using the resulting testing method. As a result, it was found that the corrosion resistance of the steel after peeling of a coating film of the coal carrier or ore/coal carrier hold was improved by adding Sb or further adding Cu and Ni and, thereby, the present invention has been completed. Meanwhile, the testing method simulating an environment in the coal carrier or ore/coal carrier hold will be described later in the example.
1. A corrosion-resistant steel for a coal carrier or ore/coal carrier hold, characterized in that the chemical composition of the steel contains C: 0.010 to 0.200 percent by mass, Si: 0.05 to 0.50 percent by mass, Mn: 0.10 to 2.0 percent by mass, P: 0.0250 percent by mass or less, S: 0.010 percent by mass or less, Al: 0.0050 to 0.10 percent by mass, Sb: 0.010 to 0.50 percent by mass, N: 0.0010 to 0.0080 percent by mass, and further comprises at least one selected from Cu: 0.010 to 1.0 percent by mass and Ni: 0.010 to 1.0 percent by mass, and further comprises optionally at least one selected from Cr: 0.050 percent by mass or less, W: 0.005 to 0.5 percent by mass, Mo: 0.005 to 0.5 percent by mass, Ti: 0.0010 to 0.030 percent by mass, Nb: 0.0010 to 0.030 percent by mass, Zr: 0.0010 to 0.030 percent by mass, V: 0.0020 to 0.20 percent by mass, Ca: 0.0005 to 0.0040 percent by mass, REM: 0.0001 to 0.0150 percent by mass, Y: 0.0001 to 0.10 percent by mass, Se: 0.0005 to 0.50 percent by mass, Te: 0.0005 to 0.50 percent by mass, and Co: 0.010 to 0.50 percent by mass, and in addition, the remainder being Fe and inevitable impurities.
2. The corrosion-resistant steel for a coal carrier or ore/coal carrier hold, according to the item 1, characterized in that in the above-described steel, Cr is 0.050 percent by mass or less.
3. The corrosion-resistant steel for a coal carrier or ore/coal carrier hold, according to item 1 or item 2, characterized by containing at least one selected from W: 0.005 to 0.5 percent by mass and Mo: 0.005 to 0.5 percent by mass in addition to the above-described steel.
4. The corrosion-resistant steel for a coal carrier or ore/coal carrier hold, according to any one of the items 1 to 3, characterized by containing at least one selected from Ti: 0.0010 to 0.030 percent by mass, Nb: 0.0010 to 0.030 percent by mass, Zr: 0.0010 to 0.030 percent by mass, and V: 0.0020 to 0.20 percent by mass in addition to the above-described steel.
5. The corrosion-resistant steel for a coal carrier or ore/coal carrier hold, according to any one of the items 1 to 4, characterized by containing Ca: 0.0005 to 0.0040 percent by mass in addition to the above-described steel.
6. The corrosion-resistant steel for a coal carrier or ore/coal carrier hold, according to any one of the items 1 to 5, characterized by containing at least one selected from REM: 0.0001 to 0.0150 percent by mass and Y: 0.0001 to 0.10 percent by mass in addition to the above-described steel.
7. The corrosion-resistant steel for a coal carrier or ore/coal carrier hold, according to any one of the items 1 to 6, characterized by containing at least one selected from Se: 0.0005 to 0.50 percent by mass, Te: 0.0005 to 0.50 percent by mass, and Co: 0.010 to 0.50 percent by mass in addition to the above-described steel.

### [Advantageous Effects of Invention]

According to the present invention, a corrosion-resistant steel for a coal carrier or ore/coal carrier hold can be obtained, wherein corrosion after peeling of a coating film can be inhibited under a cyclic wet and dry environment and a low pH environment in the coal carrier or ore/coal carrier hold.

### [Brief Description of Drawings]

[Fig. 1] Fig. 1 is a diagram showing an example of temperature-humidity cycle in a coal corrosion test.
[Fig. 2] Fig. 2 is a diagram to estimate a maximum thickness decrease of a coal carrier or ore/coal carrier hold steel 25 years later.
[Fig. 3] Fig. 3 is a diagram showing the results of S mapping after a coal corrosion test of an invention example and a comparative example on the basis of electron probe micro-analysis.

### [Description of Embodiments]

The embodiments according to the present invention will be described below. To begin with, reasons for the limitation of the chemical composition of the steel to the above-described range in the present invention will be described.

### C: 0.010 to 0.200 percent by mass

Carbon is an element effective in enhancing the strength of the steel. In the present invention, it is necessary that the content be 0.010 percent by mass or more to ensure the strength. On the other hand, if the content is more than 0.200 percent by mass, the weldability and the toughness of a heat-affected zone are degraded. Therefore, C is specified to be within the range of 0.010 to 0.200 percent by mass, and preferably within the range of 0.050 to 0.150 percent by mass.

### Si: 0.05 to 0.50 percent by mass

Silicon is added as a deoxidizing agent and is an element to enhance the strength of the steel. In the present invention, the content is specified to be 0.05 percent by mass or more. However, if the content is more than 0.50 percent by mass, the toughness of the steel is degraded. Therefore, the upper limit of Si is specified to be 0.50 percent by mass. In addition, Si forms a corrosion protection film in an acidic environment to improve corrosion resistance. In order to obtain this effect, Si is preferably within the range of 0.20 to 0.40 percent by mass.

### Mn: 0.10 to 2.0 percent by mass

Manganese is an element capable of enhancing the strength of the steel at a low cost and, furthermore, capable of preventing hot brittleness. Therefore, the content is specified to be 0.10 percent by mass or more. However, if the content is more than 2.0 percent by mass, the toughness and the weldability of the steel are degraded. Therefore, Mn is specified to be within the range of 2.0 percent by mass or less, and preferably within the range of 0.80 to 1.4 percent by mass from the viewpoint of ensuring of the strength and reduction of inclusions.

### P: 0.0250 percent by mass or less

Phosphorus is a harmful element which degrades not only the base material toughness of the steel but also the weldability and the welded portion toughness and, therefore, is desirably minimized. In particular, if the P content is more than 0.0250 percent by mass, degradation in the base material toughness and the welded portion toughness become significant. Therefore, P is specified to be 0.0250 percent by mass or less, and preferably 0.0150 percent by mass or less.

### S: 0.010 percent by mass or less

Sulfur forms MnS serving as a start point of local corrosion and degrades the local corrosion resistance. In addition, sulfur is a harmful element which degrades the toughness and the weldability of the steel and, therefore, is desirably minimized. In the present invention, S is limited to 0.010 percent by mass or less, preferably 0.007 percent by mass or less, and further preferably 0.005 percent by mass or less.

### Al: 0.0050 to 0.10 percent by mass

Aluminum is added as a deoxidizing agent. For this purpose, it is necessary that the content be 0.0050 percent by mass or more. If the content is more than 0.10 percent by mass, when welding is performed, the toughness of a welded metal portion is degraded. Therefore, Al is limited to within the range of 0.0050 to 0.10 percent by mass, and preferably 0.010 to 0.050 percent by mass.

### Sb: 0.010 to 0.50 percent by mass

When 0.010 percent by mass or more of Sb is contained as an alloy element in the steel, Sb is concentrated in the vicinity of the steel in a low pH environment. Antimony has a large hydrogen overvoltage, so that a hydrogen generation reaction is inhibited in a portion where Sb has been precipitated and the corrosion resistance is improved. Furthermore, Sb densifies corrosion products and inhibits diffusion of H₂O, O₂, SO₄²⁻, and Cl⁻ into the steel.

On the other hand, if more than 0.50 percent by mass of Sb is added, the toughness is degraded. Therefore, Sb is limited to within the range of 0.010 to 0.50 percent by mass, preferably within the range of 0.010 to 0.30 percent by mass, and further preferably within the range of 0.010 to 0.20 percent by mass.

### N: 0.0010 to 0.0080 percent by mass

Nitrogen is an element to degrade the toughness and is desirably minimized. However, it is difficult to decrease to less than 0.0010 percent by mass industrially. On the other hand, if the content is more than 0.0080 percent by mass, significant reduction in the toughness is caused. Therefore, in the present invention, N is limited to within the range of 0.0010 to 0.0080 percent by mass, and preferably 0.0010 to 0.0050 percent by mass.

Furthermore, the steel according to the present invention contains at least one selected from Cu and Ni within the following range in addition to the above-described indispensable components.

### Cu: 0.010 to 1.0 percent by mass

Copper densifies corrosion products and inhibits diffusion of H₂O, O₂, SO₄²⁻, and Cl⁻ into the steel. Consequently, the corrosion resistance of the steel is improved. This effect is exerted when the content is 0.010 percent by mass or more. However, as the amount of addition increases, the weldability and the toughness of the base material are degraded. Therefore, in the case where Cu is contained, Cu is preferably within the range of 0.010 to 1.0 percent by mass, further preferably within the range of 0.010 to 0.50 percent by mass, and still more preferably within the range of 0.010 to 0.35 percent by mass. Also, Cu forms Cu₂Sb, which is an intermetallic compound, under coexistence with Sb and, therefore, has an effect in improving the corrosion resistance.

### Ni: 0.010 to 1.0 percent by mass

Nickel densifies corrosion products and inhibits diffusion of H₂O, O₂, SO₄²⁻, and Cl⁻ into the steel as with Cu. Consequently, the corrosion resistance of the steel is improved. This effect is exerted when the content is 0.010 percent by mass or more. However, if the content is more than 1.0 percent by mass, the effect is saturated and, in addition, the cost increases. Therefore, in the case where Ni is contained, Ni is preferably within the range of 0.010 to 1.0 percent by mass, and further preferably within the range of 0.010 to 0.50 percent by mass.

The steel according to the present invention can contain Cr within the following range in addition to the above-described components.

### Cr: 0.050 percent by mass or less

Chromium is an element to cause hydrolysis in a low pH environment and, thereby, degrade the corrosion resistance. Therefore, Cr is not necessarily added. Chromium can be added to adjust the strength. However, in particular, if the content is more than 0.050 percent by mass, the corrosion resistance is degraded significantly. Therefore, in the case where Cr is contained, the content is preferably 0.050 percent by mass or less, and further preferably 0.030 percent by mass or less.

### W: 0.005 to 0.5 percent by mass and Mo: 0.005 to 0.5 percent by mass

Tungsten and molybdenum form oxoacids when being eluted from the base material, the oxoacids electrically repel anions and prevent anions from entering up to the steel surface, so that the corrosion resistance is improved. Furthermore, Mo and W improve the corrosion resistance by forming sparingly soluble corrosive materials, e.g., FeMoO₄ and FeWO₄. In order to obtain these effects, the content of each of them is preferably 0.005 percent by mass or more. However, even when addition is more than 0.5 percent by mass, not only the effect is saturated but also the cost increases. Therefore, in the case where W and Mo are contained, the content is preferably 0.5 percent by mass or less, and further preferably 0.010 to 0.3 percent by mass.

The steel according to the present invention can further contain at least one selected from Ti, Nb, Zr, and V within the following range in addition to the above-described components for the purpose of enhancing the strength.

At least one selected from Ti: 0.0010 to 0.030 percent by mass, Nb: 0.0010 to 0.030 percent by mass, Zr: 0.0010 to 0.030 percent by mass, and V: 0.0020 to 0.20 percent by mass

Each of Ti, Nb, Zr, and V is an element to enhance the strength of the steel and can be selected and contained in accordance with the required strength. In order to obtain such an effect, the contents of Ti, Nb, and Zr are preferably 0.0010 percent by mass or more and the content of V is preferably 0.0020 percent by mass or more. However, if each of the content of Ti, Nb, and Zr is more than 0.030 percent by mass or the content of V is more than 0.20 percent by mass, the toughness is degraded. Therefore, in the case where Ti, Nb, Zr, and V are contained, the content of each of them is preferably within the above-described range, and Ti: 0.0050 to 0.020 percent by mass, Nb: 0.0050 to 0.020 percent by mass, Zr: 0.0050 to 0.020 percent by mass, and V: 0.0050 to 0.10 percent by mass are further preferable.

The steel according to the present invention can contain Ca within the following range in addition to the above-described components.

### Ca: 0.0005 to 0.0040 percent by mass

Calcium is an element to control the forms of inclusions and enhance the ductility and the toughness of the steel. In order to exert such effects, the content is preferably at least 0.0005 percent by mass. However, if the content is too large, coarse inclusions are formed and the toughness of the base material is degraded. Therefore, in the case where Ca is contained, the upper limit is specified to be preferably 0.0040 percent by mass, and 0.0010 to 0.0030 percent by mass is further preferable.

The steel according to the present invention can further contain at least one selected from REM and Y within the following range in addition to the above-described components for the purpose of improving the toughness.

### REM: 0.0001 to 0.0150 percent by mass and Y: 0.0001 to 0.10 percent by mass

Each of REM (rare earth metal) and Y is an element to enhance the toughness of a heat-affected zone and can be contained as necessary. This effect is obtained when the content of each of REM and Y is 0.0001 percent by mass or more. However, if the content of REM is more than 0.0150 percent by mass or the content of Y is more than 0.10 percent by mass, degradation in the toughness is caused. Therefore, in the case where REM and Y are contained, the content of each of them is preferably within the above-described range.

The steel according to the present invention can further contain at least one selected from Se, Te, and Co within the following range in addition to the above-described components for the purpose of enhancing the strength.

At least one of Se: 0.0005 to 0.50 percent by mass, Te: 0.0005 to 0.50 percent by mass, and Co: 0.010 to 0.50 percent by mass
Selenium, tellurium, and cobalt are elements to enhance the strength of the steel and can be contained as necessary. In order to obtain this effect, the contents of Se and Te are preferably 0.0005 percent by mass or more and the content of Co is preferably 0.010 percent by mass or more. However, if each of the contents of Se, Te, and Co is more than 0.50 percent by mass, the toughness and the weldability are degraded. Therefore, in the case where Se, Te, and Co are contained, the contents are preferably specified to be within the above-described range.

Among the chemical components according to the present invention, the components other than those described above are Fe and inevitable impurities. However, components other than those described above may be contained within the bounds of not impairing the effects of the present invention. For example, Mg: 0.0001 to 0.010 percent by mass can be contained for the purpose of improving the toughness.

On the other hand, as shown in the examples later, even when Sn is contained in stead of Sb, an effect of reducing the corrosion weight loss and the maximum pitting corrosion depth is not exerted. Furthermore, coexistence of Sn with Cu lowers the melting point of Cu and further reduces the solid solubility into iron, so that Cu is precipitated at grain boundaries on the steel surface and hot brittleness is caused. Consequently, Sn is not added, although the content of less than 0.005 percent by mass is permissible as an impurity because hot brittleness is not caused.

Next, a preferred method for manufacturing the corrosion-resistant steel according to the present invention will be described, although the present invention can be applied to manufacturing methods other than this.

A steel produced by continuous casting or the like is hot-rolled on an "as is" basis or while reheat is performed after cooling. The heat treatment condition to exhibit the corrosion resistance is not specifically limited, but it is preferable that an appropriate reduction ratio be ensured from the viewpoint of the mechanical property. If the finishing temperature of hot rolling is lower than 750°C, deformation resistance increases and a defective shape is caused. Therefore, the finishing temperature is specified to be preferably 750°C or higher.

For example, a steel having a tensile strength of 490 MPa-grade or more can be produced by specifying the finishing temperature to be 750°C or higher and, thereafter, controlling the cooling rate in such a way that cooling to 600°C or lower is performed at a cooling rate of 150°C/min or more.

### [EXAMPLES]

A steel to contain components shown in Table 1 was smelted with a vacuum melting furnace or smelted with a converter and, thereafter, a slab was produced by continuous casting. Subsequently, the slab was put into a furnace and was heated to 1,200°C. A steel plate having a thickness of 25 mm was produced by hot rolling at a finishing temperature of 800°C.

The present inventors examined the mechanism of an occurrence of pitting corrosion which has a largest influence on breakage of ship among corrosion in a coal carrier or ore/coal carrier hold. The results were as described below. The side shell of a bulk carrier is a single-hull, and a cargo and the seawater is separated by only a plate of steel. Consequently, dew condensation water is generated on the hold side shell because of a temperature difference between the seawater and the inside of the hold, so that the surfaces of the steel and the coal are wetted and H₂SO₄-derived substances adsorbed to the coal surface are leached into a water film. Pitting corrosion proceeds under the coal forming a meniscus, and H⁺ is consumed in corrosion of the steel, so that the H⁺ concentration is reduced in the meniscus portion. On the other hand, the coal surface is rich in H⁺, and a difference in the H⁺ concentration occurs between the coal surface and the meniscus portion. It is considered that the difference in the chemical potential serves as a driving force and H⁺ is fed from the coal surface to the meniscus portion. Then, in a drying step, unreacted H⁺ adheres to the coal surface again and is used for a corrosion reaction in the next dew condensation step. This steps occur over a long-term cycle, corrosion is facilitated in the meniscus portion, and pitting corrosion proceeds. In order to perform laboratory simulation of pitting corrosion in a coal carrier or ore/coal carrier hold, the following condition was employed on the basis of the present mechanism.

### (EXAMPLE 1)

Initially, in order to measure the maximum pitting corrosion depth by using the steel plate shown in Table 1, an example was obtained in the procedure described below (the present testing method is referred to as Corrosion test a).
A test piece of 5 mm^{t} × 50 mm^{W} × 75 mm^{L} was taken from the steel plate containing components shown in Table 1. The surface of the test piece was subjected to shot blasting to remove scales and oil contents on the surface. The resulting surface was specified to be a test surface and the corrosion resistance of the steel after peeling of a coating film was evaluated. The back and the end surface were coated with silicon base adhesive tape, the test piece was fit into an acrylic cell, and 5 g of coal was laid thereon. A temperature-humidity cycle of Atmosphere A (temperature 60°C, humidity 95%, and 20 hours) ↔ Atmosphere B (temperature 30°C, humidity 95%, and 3 hours) with transition time of 0.5 hours, as shown in Fig. 1, was applied for 28 days with a temperature and humidity chamber. Here, the symbol "↔" is used in the sense of repetition (the same goes hereafter). In this regard, the coal employed was specified in such a way that when 5 g of coal was weighed and immersed in 100 ml of distilled water at ambient temperature for 2 hours and, thereafter, filtration was performed, the pH of a liquid leached from the coal and diluted to 200 ml became 3.0. The present example was allowed to simulate the temperature-humidity environment and the dew condensation situation having a large influence on corrosion in a coal carrier or ore/coal carrier hold by performing an examination under such conditions. After the test, rust of each test piece was peeled by using a rust peeling liquid, and the amount of weight decrease of the steel was measured and taken as the amount of corrosion. Also, the resulting maximum pitting corrosion depth was measured with a depth meter. The results thereof are shown in Table 2.

As is clear from Table 2, in all Test Nos. 4-a to 9-a, 12-a to 16-a, 18-a, 19-a and 21-a to 27-a (the numerical part of Test No. and Steel plate No. agreed with each other, the same goes hereafter) and Nos. 35-a to 40-a which were the invention examples, both the weight decrease and the maximum pitting corrosion depth were good as compared with those of comparative materials, the weight decrease was controlled to be 2.5 g or less, and the maximum pitting corrosion depth was controlled to be 0.30 mm or less. On the other hand, in Test Nos. 28-a and 29-a which were comparative materials, more than 0.050 percent by mass of Cr was contained and in Test Nos. 30-a and 32-a, Sb was not contained but Sn was contained, so that the weight decrease was 2.7 g or more and the maximum pitting corrosion depth was 0.35 mm or more in all cases. In this regard, in Test No. 31-a, Sb was not contained and, therefore, the weight decrease was 2.71 g and the maximum pitting corrosion depth was 0.34 mm, so that the corrosion resistance was inferior to the corrosion resistance of the invention examples in spite of the fact that the amount of elements other than Sb were within the scope of the present invention.

### (EXAMPLE 2)

Next, an example to estimate a maximum thickness decrease 25 years later will be described. As with Example 1, a test piece of 5 mm^{t} × 50 mm^{W} × 75 mm^{L} was taken from the steel plate shown in Table 1. The surface of the test piece was subjected to shot blasting to remove scales and oil contents on the surface. The resulting surface was specified to be a test surface and the corrosion resistance of the steel after peeling of a coating film was evaluated. The back and the end surface were coated with silicon base adhesive tape, the test piece was fit into an acrylic cell, and 5 g of coal was laid thereon. A temperature-humidity cycle of Atmosphere A (temperature 60°C, humidity 95%, and 20 hours) ↔ Atmosphere B (temperature 30°C, humidity 95%, and 3 hours) with transition time of 0.5 hours, as shown in Fig. 1, was applied for 28, 56, 84, 168, or 336 days with a temperature and humidity chamber (the present testing method is referred to as Corrosion test b).

In this regard, the coal employed was specified in such a way that when 5 g of coal was weighed and immersed in 100 ml of distilled water at ambient temperature for 2 hours and, thereafter, filtration was performed, the pH of a liquid leached from the coal and diluted to 200 ml became 3.0. The present example was allowed to simulate the temperature-humidity environment and the dew condensation situation having a large influence on corrosion in a coal carrier or ore/coal carrier hold by performing an examination under such conditions. After the test, rust of each test piece was peeled by using a rust peeling liquid, and the maximum pitting corrosion depth in each time period was measured. However, the value of maximum pitting corrosion depth increased as a subject area increased. Then, in order to predict the maximum pitting corrosion depth in each time period of an actual ship, the maximum pitting corrosion depth in an area equivalent to the actual ship hold area was calculated from the measurement value in the present test piece area by using extreme value statistics. Here, the hold side frame portion, which is an application area of the present development steel, is corroded from both surfaces. Therefore, the maximum pitting corrosion depth in each time period was doubled, and the maximum thickness decrease 25 years later, which was a life time of ship, was estimated by extrapolation of those values. The results thereof are shown in Table 3. The criteria of the maximum thickness decrease 25 years later were specified to be 4.0 mm on the basis of the steel plate renewal guideline of RULES FOR THE SURVEY AND CONSTRUCTION OF STEEL SHIPS PART CSR-B (IACS common structure rule for bulk carrier) on the precondition that the plate thickness of the application area was 15 to 20 mm, the corrosion allowance was 3.5 to 4.0 mm, and the voluntary thickness addition was 0.5 mm.

In addition, S mapping of rust cross-sections of Invention example No. 37-b and Comparative example No. 44-b after the test for 84 days were performed on the basis of the electron probe micro-analysis. As for the electron probe micro-analysis, EPMA1600 produced by SHIMADZU CORPORATION was used, and a region of 100 x 100 µm was measured at acceleration voltage: 20 kV, beam diameter: 1 µm, and 0.4 µm pitch in the X and Y directions.

Fig. 2 shows a graph to estimate a maximum thickness decrease 25 years later. Here, the maximum thickness decrease refers to the thickness of steel plate in the portion which has been lost by local corrosion and at which the thickness decrease from the as-built thickness of a ship is maximum. Invention example No. 37-b and Comparative example No. 44-b are described. The maximum thickness decrease in each time period used for forming Fig. 2 was as described below in Invention example No. 37-b. 28 days: 0.85 mm, 56 days: 1.11 mm, 84 days: 1.28 mm, 168 days: 1.36 mm, and 336 days: 1.47 mm. In this regard, those in Comparative example No. 44-b were as described below. 28 days: 0.96 mm, 56 days: 1.39 mm, 84 days: 1.62 mm, 168 days: 1.91 mm, and 336 days: 2.11 mm. Meanwhile, in all of Test Nos. 4-b to 9-a, 12-a to 16-a, 18-a, 19-a and 21-a to 27-b and Test Nos. 35-b to 40-b of Invention examples shown in Table 3, estimated maximum thickness decreases 25 years later were less than or equal to 4.0 mm, which was the criteria. In this regard, No. 31-b, in which only addition of Sb was out of the present claim, did not satisfy the criteria. Therefore, it is clear that Sb has a large influence on corrosion protection in the present environment.

Also, Fig. 3 shows the results of S mapping of rust portion cross-sections after 84 days in Corrosion test b on the basis of the electron probe micro-analysis. In Comparative example No. 44-b, an interface layer rich in S is present between a rust layer and a steel, whereas in Invention example No. 37-b, an interface layer rich in S is hardly observed. Consequently, it is estimated that in Invention example, SO₄²⁻ permeation to rust/steel interface is inhibited by densification of rust due to Sb and electrical repulsion of SO₄²⁻ due to an oxoacid of W. Accordingly, it is clear that the present invention is a steel which forms a rust layer to inhibit SO₄²⁻ permeation in a coal carrier or ore/coal carrier hold environment.

As described above, the effects of the present invention were ascertained. In the present example, the method shown in Fig. 1 was employed as the testing method simulating the coal carrier or ore/coal carrier hold environment, and results very consistent with those in the case where evaluation was performed on the basis of placement in an actual coal carrier or ore/coal carrier hold were obtained. In this regard, the conditions of Atmospheres A and B, the transition times, the cycle, the method for adjusting the coal, and the conditions, e.g., the value of pH of the liquid leached from the coal, are not limited to the above-described examples and can be changed appropriately in accordance with the use environment of the steel in the hold.

### [Industrial Applicability]

The steel according to the present invention can be used as a constituent member of a coal carrier or ore/coal carrier hold, where the coating film is peeled easily because of mechanical damages by coals and ores, and the steel is exposed to a cyclic wet and dry environment and a low pH environment.
[Table 1-1]

**Table 1-1 (mass%)**

| Steel plate No. | C | Si | Mn | P | S | Al | Sb | Cu | Ni | Cr | Sn | Mo | W | Remarks |
|---|---|---|---|---|---|---|---|---|---|---|---|---|---|---|
| 1 | 0.144 | 0.27 | 1.06 | 0.012 | 0.004 | 0.034 | 0.01 | - | - | - | - | - | - | Reference example |
| 2 | 0.145 | 0.28 | 1.07 | 0.012 | 0.004 | 0.032 | 0.11 | - | - | - | - | - | - | Reference example |
| 3 | 0.142 | 0.28 | 1.07 | 0.011 | 0.004 | 0.032 | 0.49 | - | - | - | - | - | - | Reference example |
| 4 | 0.145 | 0.28 | 1.06 | 0.011 | 0.004 | 0.036 | 0.10 | 0.01 | - | - | - | - | - | Invention example |
| 5 | 0.143 | 0.28 | 1.06 | 0.011 | 0.004 | 0.035 | 0.10 | 0.10 | - | - | - | - | - | Invention example |
| 6 | 0.142 | 0.29 | 1.07 | 0.012 | 0.004 | 0.034 | 0.11 | 0.98 | - | - | - | - | - | Invention example |
| 7 | 0.145 | 0.28 | 1.07 | 0.012 | 0.004 | 0.033 | 0.10 | - | 0.01 | - | - | - | - | Invention example |
| 8 | 0.144 | 0.28 | 1.06 | 0.012 | 0.004 | 0.034 | 0.09 | - | 0.11 | - | - | - | - | Invention example |
| 9 | 0.143 | 0.28 | 1.06 | 0.011 | 0.004 | 0.048 | 0.11 | - | 0.96 | - | - | - | - | Invention example |
| 10 | 0.141 | 0.29 | 1.06 | 0.012 | 0.004 | 0.033 | 0.10 | - | - | 0.010 | - | - | - | Reference example |
| 11 | 0.146 | 0.28 | 1.07 | 0.012 | 0.004 | 0.035 | 0.11 | - | - | 0.030 | - | - | - | Reference example |
| 12 | 0.146 | 0.28 | 1.07 | 0.012 | 0.004 | 0.037 | 0.11 | 0.25 | 0.11 | - | - | - | - | Invention example |
| 13 | 0.103 | 0.25 | 0.46 | 0.013 | 0.007 | 0.048 | 0.11 | 0.30 | 0.17 | - | - | - | - | Invention example |
| 14 | 0.146 | 0.24 | 1.06 | 0.012 | 0.004 | 0.031 | 0.10 | 0.32 | 0.15 | 0.020 | - | - | - | Invention example |
| 15 | 0.144 | 0.28 | 1.08 | 0.011 | 0.004 | 0.032 | 0.10 | 0.35 | 0.11 | - | - | 0.10 | - | Invention example |
| 16 | 0.146 | 0.27 | 1.06 | 0.011 | 0.004 | 0.030 | 0.11 | 0.35 | 0.10 | - | - | - | 0.11 | Invention example |
| 17 | 0.145 | 0.28 | 1.07 | 0.012 | 0.004 | 0.032 | 0.11 | - | - | - | - | - | - | Reference example |
| 18 | 0.141 | 0.29 | 1.06 | 0.012 | 0.004 | 0.030 | 0.12 | 0.19 | - | - | - | - | - | Invention example |
| 19 | 0.146 | 0.24 | 1.08 | 0.010 | 0.005 | 0.033 | 0.10 | - | 0.31 | - | - | - | - | Invention example |
| 20 | 0.142 | 0.28 | 1.07 | 0.011 | 0.004 | 0.034 | 0.31 | - | - | 0.010 | - | - | - | Reference example |
| 21 | 0.101 | 0.25 | 0.49 | 0.013 | 0.007 | 0.048 | 0.11 | 0.35 | 0.21 | - | - | - | - | Invention example |
| 22 | 0.102 | 0.25 | 1.08 | 0.010 | 0.005 | 0.032 | 0.11 | 0.20 | - | 0.011 | - | - | - | Invention example |

[Table 1-2]

**Table 1-2 (mass%)**

| Steel plate No. | Ti | Nb | Zr | V | Ca | REM | Y | Se | Te | Co | N | O | Remarks |
|---|---|---|---|---|---|---|---|---|---|---|---|---|---|
| 1 | - | - | - | - | - | - | - | - | - | - | 0.0029 | 0.0012 | Reference example |
| 2 | - | - | - | - | - | - | - | - | - | - | 0.0027 | 0.0011 | Reference example |
| 3 | - | - | - | - | - | - | - | - | - | - | 0.0029 | 0.0015 | Reference example |
| 4 | - | - | - | - | - | - | - | - | - | - | 0.0026 | 0.0024 | Invention example |
| 5 | - | - | - | - | - | - | - | - | - | - | 0.0026 | 0.0017 | Invention example |
| 6 | - | - | - | - | - | - | - | - | - | - | 0.0029 | 0.0021 | Invention example |
| 7 | - | - | - | - | - | - | - | - | - | - | 0.0020 | 0.0013 | Invention example |
| 8 | - | - | - | - | - | - | - | - | - | - | 0.0022 | 0.0013 | Invention example |
| 9 | - | - | - | - | - | - | - | - | - | - | 0.0038 | 0.0018 | Invention example |
| 10 | - | - | - | - | - | - | - | - | - | - | 0.0020 | 0.0013 | Reference example |
| 11 | - | - | - | - | - | - | - | - | - | - | 0.0026 | 0.0017 | Reference example |
| 12 | - | - | - | - | - | - | - | - | - | - | 0.0023 | 0.0021 | Invention example |
| 13 | - | - | - | - | - | - | - | - | - | - | a.oo3s | 0.0018 | Invention example |
| 14 | - | - | - | - | - | - | - | - | - | - | 0.0021 | 0.0010 | Invention example |
| 15 | - | - | - | - | - | - | - | - | - | - | 0.0028 | 0.0019 | Invention example |
| 16 | - | - | - | - | - | - | - | - | - | - | 0.0025 | 0.0013 | Invention example |
| 17 | 0.010 | - | - | - | - | - | - | - | - | - | 0.0027 | 0.0011 | Reference example |
| 18 | - | 0.009 | - | - | - | - | - | - | - | - | 0.0021 | 0.0010 | Invention example |
| 19 | - | - | 0.011 | - | - | - | - | - | - | - | 0.0020 | 0.0013 | Invention example |
| 20 | - | - | - | 0.01 | - | - | - | - | - | - | 0.0022 | 0.0013 | Reference example |
| 21 | - | - | - | - | 0.002 | - | - | - | - | - | 0.0038 | 0.0018 | Invention example |
| 22 | - | - | - | - | - | 0.005 | - | - | - | - | 0.0027 | 0.0011 | Invention example |

[Table 1-3]

**Table 1-3 (mass%)**

| Steel plate No. | C | Si | Mn | P | S | Al | Sb | Cu | Ni | Cr | Sn | Mo | W | Remarks |
|---|---|---|---|---|---|---|---|---|---|---|---|---|---|---|
| 23 | 0-030 | 0.50 | 1.01 | 0.011 | 0.005 | 0.033 | 0.32 | - | 0.19 | 0.031 | - | - | - | Invention example |
| 24 | 0.144 | 0.24 | 1.03 | 0.012 | 0.004 | 0.034 | 0.10 | 0.21 | 0.10 | - | - | - | - | Invention example |
| 25 | 0.031 | 0.48 | 0.94 | 0.008 | 0.007 | 0.037 | 0.11 | 0.10 | 0.05 | - | - | - | - | Invention example |
| 26 | 0.030 | 0.50 | 0.93 | 0.008 | 0.006 | 0.039 | 0.30 | 0.1 | - | 0.010 | - | - | - | Invention example |
| 27 | 0.146 | 0.24 | 1.06 | 0.012 | 0.004 | 0.045 | 0.10 | 0.20 | 0.10 | 0.010 | - | - | - | Invention example |
| 28 | 0.031 | 0.45 | 0.93 | 0.008 | 0.006 | 0.038 | 0.09 | 0.01 | 0.01 | 0.220 | - | - | - | Comparative example |
| 29 | 0.101 | 0.45 | 0.94 | 0.008 | 0.006 | 0.037 | 0.10 | 0.01 | 0.01 | 0.710 | - | - | - | Comparative example |
| 30 | 0.139 | 0.28 | 1.05 | 0.012 | 0.004 | 0.032 | - | - | 0.01 | - | 0.35 | - | - | Comparative example |
| 31 | 0.144 | 0.28 | 1.01 | 0.010 | 0.003 | 0.033 | - | 0.20 | 0.11 | 0.011 | - | 0.04 | - | Comparative example |
| 32 | 0.159 | 0.28 | 1.12 | 0.018 | 0.002 | 0.027 | - | 0.21 | 0.01 | 0.020 | 0.10 | - | - | Comparative example |
| 33 | 0.144 | 0.27 | 1.06 | 0.012 | 0.004 | 0.034 | 0.02 | - | - | - | - | - | - | Reference example |
| 34 | 0.146 | 0.28 | 1.07 | 0.012 | 0.004 | 0.035 | 0.11 | - | - | 0.030 | - | - | - | Reference example |
| 35 | 0.144 | 0.28 | 1.08 | 0.011 | 0.004 | 0.032 | 0.10 | 0.35 | 0.11 | - | - | 0.10 | - | Invention example |
| 36 | 0.146 | 0.24 | 1.08 | 0.010 | 0.005 | 0.033 | 0.10 | - | 0.31 | - | - | - | - | Invention example |
| 37 | 0.144 | 0.30 | 1.03 | 0.007 | 0.002 | 0.034 | 0.10 | 0.21 | 0.10 | - | - | - | 0.05 | Invention example |
| 38 | 0.031 | 0.48 | 0.94 | 0.008 | 0.007 | 0.037 | 0.11 | 0.16 | 0.05 | - | - | - | 0.05 | Invention example |
| 39 | 0.030 | 0.50 | 0.93 | 0.008 | 0.006 | 0.039 | 0.11 | 0.20 | 0.10 | - | - | - | 0.45 | Invention example |
| 40 | 0.146 | 0.24 | 1.06 | 0.012 | 0.004 | 0.045 | 0.10 | 0.20 | 0.10 | 0.010 | - | - | - | Invention example |
| 41 | 0.031 | 0.45 | 0.93 | 0.008 | 0.006 | 0.038 | - | 0.01 | 0.01 | 0.220 | - | - | 0.05 | Comparative example |
| 42 | 0.101 | 0.45 | 0.94 | 0.008 | 0.006 | 0.037 | - | 0.01 | 0.01 | 0.710 | - | - | 0.10 | Comparative example |
| 43 | 0.139 | 0.28 | 1.05 | 0.012 | 0.004 | 0.032 | - | - | 0.01 | - | - | 0.35 | - | Comparative example |
| 44 | 0.159 | 0.28 | 1.12 | 0.018 | 0.002 | 0.027 | - | 0.02 | 0.01 | 0.020 | 0.10 | - | - | Comparative example |

[Table 1-4]

**Table 1-4 (mass%)**

| Steel plate No. | Ti | Nb | Zr | V | Ca | REM | Y | Se | Te | Co | N | O | remarks |
|---|---|---|---|---|---|---|---|---|---|---|---|---|---|
| 23 | 0.011 | - | - | - | - | - | 0.006 | - | - | - | 0.0020 | 0.0013 | Invention example |
| 24 | - | 0.010 | - | - | - | - | - | 0.001 | - | - | 0.0022 | 0.0013 | Invention example |
| 25 | - | - | - | - | 0.002 | - | - | - | 0.0011 | - | 0.0023 | 0.0022 | Invention example |
| 26 | - | - | 0.012 | - | - | - | 0.005 | - | - | 0.014 | 0.0025 | 0.0013 | Invention example |
| 27 | 0.01 | - | - | 0.001 | 0.001 | - | - | - | - | 0.009 | 0.0028 | 0.0018 | Invention example |
| 28 | - | - | - | - | - | - | - | - | - | - | 0.0044 | 0.0018 | Comparative example |
| 29 | - | - | - | - | - | - | - | - | - | - | 0.0043 | 0.0014 | Comparative example |
| 30 | - | - | - | - | - | - | - | - | - | - | 0.0030 | 0.0016 | Comparative example |
| 31 | 0.011 | 0.013 | - | - | 0.002 | - | - | - | - | 0.008 | 0.0026 | 0.0018 | Comparative example |
| 32 | 0.015 | 0.010 | - | - | - | - | - | - | - | - | 0.0029 | 0.0013 | Comparative example |
| 33 | - | - | - | - | - | - | - | - | - | - | 0.0029 | 0.0012 | Reference example |
| 34 | - | - | - | - | - | - | - | - | 0.0011 | - | 0.0026 | 0.0017 | Reference example |
| 35 | - | - | - | - | - | - | - | - | - | 0.014 | 0.0028 | 0.0019 | Invention example |
| 36 | - | - | 0.011 | - | - | - | - | 0.001 | - | - | 0.0020 | 0.0013 | Invention example |
| 37 | 0.011 | 0.015 | - | - | - | - | - | - | - | - | 0.0022 | 0.0013 | Invention example |
| 38 | 0.011 | 0.015 | - | - | 0.002 | - | - | - | 0.0011 | - | 0.0023 | 0.0022 | Invention example |
| 39 | 0.011 | - | - | - | - | - | 0.005 | - | - | - | 0.0025 | 0.0013 | Invention example |
| 40 | 0,012 | - | - | 0.001 | 0.001 | - | - | - | - | - | 0.0028 | 0.0018 | Invention example |
| 41 | - | - | - | - | - | - | - | - | - | - | 0.0044 | 0.0018 | Comparative example |
| 42 | - | - | - | - | - | - | - | - | - | - | 0.0043 | 0.0014 | Comparative example |
| 43 | - | - | - | - | - | - | - | - | - | - | 0.0030 | 0.0016 | Comparative example |
| 44 | 0.015 | 0.010 | - | - | - | - | - | - | - | - | 0.0029 | 0.0013 | Comparative example |

[Table 2-1]

**Table 2-1**

| Test No. | Steel plate No. | Weight decrease (g) | Maximum pitting corrosion depth (mm) | Remarks |
|---|---|---|---|---|
| No.1 - a | 1 | 2.49 | 0.28 | Reference example |
| No.2 - a | 2 | 2.37 | 0.27 | Reference example |
| No.3 - a | 3 | 2.19 | 0.24 | Reference example |
| No.4 - a | 4 | 2.23 | 0.24 | Invention example |
| No.5 - a | 5 | 2.05 | 0.23 | Invention example |
| No.6 - a | 6 | 1.92 | 0.23 | Invention example |
| No.7 - a | 7 | 2.31 | 0.25 | Invention example |
| No.8 - a | 8 | 2.11 | 0.23 | Invention example |
| No.9 - a | 9 | 2.02 | 0.23 | Invention example |
| No.10 - a | 10 | 2.38 | 0.26 | Reference example |
| No.11 - a | 11 | 2.43 | 0.28 | Reference example |
| No.12 - a | 12 | 2.02 | 0.26 | Invention example |
| No.13 - a | 13 | 1.94 | 0.22 | Invention example |
| No.14 - a | 14 | 1.96 | 0.24 | Invention example |
| No.15 - a | 15 | 1.99 | 0.23 | Invention example |
| No.16 - a | 16 | 1.95 | 0.22 | Invention example |
| No.17 - a | 17 | 2.35 | 0.25 | Reference example |
| No.18 - a | 18 | 2.24 | 0.23 | Invention example |
| No.19 - a | 19 | 2.18 | 0.23 | Invention example |
| No.20 - a | 20 | 2.17 | 0.24 | Reference example |
| No.21 - a | 21 | 1.97 | 0.23 | Invention example |
| No.22 - a | 22 | 2.25 | 0.24 | Invention example |
| No.23 - a | 23 | 2.28 | 0.26 | Invention example |
| No.24 - a | 24 | 1.99 | 0.24 | Invention example |
| No.25 - a | 25 | 2.02 | 0.24 | Invention example |
| No.26 - a | 26 | 1.91 | 0.22 | Invention example |
| No.27 - a | 27 | 1.98 | 0.23 | Invention example |
| No.28 - a | 28 | 3.28 | 0.38 | Comparative example |
| No.29 - a | 29 | 3.49 | 0.38 | Comparative example |
| No.30 - a | 30 | 3.11 | 0.45 | Comparative example |
| No.31 - a | 31 | 2.71 | 0.34 | Comparative example |
| No.32 - a | 32 | 2.74 | 0.35 | Comparative example |

[Table 2-2]

**Table 2-2**

| Test No. | Steel plate No. | Weight decrease (g) | Maximum pitting corrosion depth (mm) | Remarks |
|---|---|---|---|---|
| No.33 - a | 33 | 2.45 | 0.28 | Reference example |
| No.34 - a | 34 | 2.40 | 0.27 | Reference example |
| No.35 - a | 35 | 2.00 | 0.24 | Invention example |
| No.36 - a | 36 | 2.20 | 0.24 | Invention example |
| No.37 - a | 37 | 2.24 | 0.25 | Invention example |
| No.38 - a | 38 | 2.31 | 0.25 | Invention example |
| No.39 - a | 39 | 2.26 | 0.25 | Invention example |
| No.40 - a | 40 | 2.29 | 0.26 | Invention example |
| No.41 - a | 41 | 3.11 | 0.35 | Comparative example |
| No.42 - a | 42 | 3.30 | 0.36 | Comparative example |
| No.43 - a | 43 | 2.72 | 0.32 | Comparative example |
| No.44 - a | 44 | 2.99 | 0.40 | Comparative example |

[Table 3-1]

**Table 3-1**

| Test No. | Steel plate No. | Estimated value of maximum thickness decrease 25 years later (mm) | Remarks |
|---|---|---|---|
| No.1 - b | 1 | 3.96 | Reference example |
| No.2 - b | 2 | 3.46 | Reference example |
| No.3 - b | 3 | 3.09 | Reference example |
| No.4 - b | 4 | 3.36 | Invention example |
| No.5 - b | 5 | 3.23 | Invention example |
| No.6 - b | 6 | 3.07 | Invention example |
| No.7 - b | 7 | 3.42 | Invention example |
| No.8 - b | 8 | 3.31 | Invention example |
| No.9 - b | 9 | 3.19 | Invention example |
| No.10 - b | 10 | 3.55 | Reference example |
| No.11 - b | 11 | 3.71 | Reference example |
| No.12 - b | 12 | 3.25 | Invention example |
| No.13 - b | 13 | 3.19 | Invention example |
| No.14 - b | 14 | 3.21 | Invention example |
| No.15 - b | 15 | 3.14 | Invention example |
| No.16 - b | 16 | 3.09 | Invention example |
| No.17 - b | 17 | 3.50 | Reference example |
| No.18 - b | 18 | 3.19 | Invention example |
| No.19 - b | 19 | 3.27 | Invention example |
| No.20 - b | 20 | 3.42 | Reference example |
| No.21 - b | 21 | 3.16 | Invention example |
| No.22 - b | 22 | 3.39 | Invention example |
| No.23 - b | 23 | 3.41 | Invention example |
| No.24 - b | 24 | 3.30 | Invention example |
| No.25 - b | 25 | 3.19 | Invention example |
| No.26 - b | 26 | 3.13 | Invention example |
| No.27 - b | 27 | 3.21 | Invention example |
| No.28 - b | 28 | 6.01 | Comparative example |
| No.29 - b | 29 | 7.90 | Comparative example |
| No.30 - b | 30 | 6.66 | Comparative example |
| No.31 - b | 31 | 4.69 | Comparative example |
| No.32 - b | 32 | 5.93 | Comparative example |

[Table 3-2]

**Table 3-2**

| Test No. | Steel plate No. | Estimated value of maximum thickness decrease 25 years later (mm) | Remarks |
|---|---|---|---|
| No.33 - b | 33 | 3.94 | Reference example |
| No.34 - b | 34 | 3.69 | Reference example |
| No.35 - b | 35 | 3.11 | Invention example |
| No.36 - b | 36 | 3.24 | Invention example |
| No.37 - b | 37 | 3.12 | Invention example |
| No.38 - b | 38 | 3.19 | Invention example |
| No.39 - b | 39 | 3.22 | Invention example |
| No.40 - b | 40 | 3.26 | Invention example |
| No.41 - b | 41 | 5.77 | Comparative example |
| No.42 - b | 42 | 7.55 | Comparative example |
| No.43 - b | 43 | 5.56 | Comparative example |
| No.44 - b | 44 | 6.33 | Comparative example |

## Claims

1. A corrosion-resistant steel for a coal carrier or ore/coal carrier hold, wherein the chemical composition of the steel consists of C: 0.010 to 0.200 percent by mass, Si: 0.05 to 0.50 percent by mass, Mn: 0.10 to 2.0 percent by mass, P: 0.0250 percent by mass or less, S: 0.010 percent by mass or less, Al: 0.0050 to 0.10 percent by mass, Sb: 0.010 to 0.50 percent by mass, N: 0.0010 to 0.0080 percent by mass, and further comprises at least one selected from Cu: 0.010 to 1.0 percent by mass and Ni: 0.010 to 1.0 percent by mass, and further comprises optionally at least one selected from Cr: 0.050 percent by mass or less, W: 0.005 to 0.5 percent by mass, Mo: 0.005 to 0.5 percent by mass, Ti: 0.0010 to 0.030 percent by mass, Nb: 0.0010 to 0.030 percent by mass, Zr: 0.0010 to 0.030 percent by mass, V: 0.0020 to 0.20 percent by mass, Ca: 0.0005 to 0.0040 percent by mass, REM: 0.0001 to 0.0150 percent by mass, Y: 0.0001 to 0.10 percent by mass, Se: 0.0005 to 0.50 percent by mass, Te: 0.0005 to 0.50 percent by mass, and Co: 0.010 to 0.50 percent by mass, and in addition, the remainder being Fe and inevitable impurities.

2. The corrosion-resistant steel for a coal carrier or ore/coal carrier hold, according to Claim 1, wherein in the steel, Cr is 0.050 percent by mass or less.

3. The corrosion-resistant steel for a coal carrier or ore/coal carrier hold, according to a Claim 1 or Claim 2, comprising at least one selected from W: 0.005 to 0.5 percent by mass and Mo: 0.005 to 0.5 percent by mass in addition to the steel.

4. The corrosion-resistant steel for a coal carrier or ore/coal carrier hold, according to any one of Claims 1 to 3, comprising at least one selected from Ti: 0.0010 to 0.030 percent by mass, Nb: 0.0010 to 0.030 percent by mass, Zr: 0.0010 to 0.030 percent by mass, and V: 0.0020 to 0.20 percent by mass in addition to the steel.

5. The corrosion-resistant steel for a coal carrier or ore/coal carrier hold, according to any one of Claims 1 to 4, comprising Ca: 0.0005 to 0.0040 percent by mass in addition to the steel.

6. The corrosion-resistant steel for a coal carrier or ore/coal carrier hold, according to any one of Claims 1 to 5, comprising at least one selected from REM: 0.0001 to 0.0150 percent by mass and Y: 0.0001 to 0.10 percent by mass in addition to the steel.

7. The corrosion-resistant steel for a coal carrier or ore/coal carrier hold, according to any one of Claims 1 to 6, comprising at least one selected from Se: 0.0005 to 0.50 percent by mass, Te: 0.0005 to 0.50 percent by mass, and Co: 0.010 to 0.50 percent by mass in addition to the steel.

## Patentansprüche

1. Korrosionsbeständiger Stahl für einen Kohletransporter oder Erz-/Kohle-Transporteraufnahme, wobei
die chemische Zusammensetzung des Stahls aus C: 0,010 bis 0,200 Massenprozent, Si: 0,05 bis 0,50 Massenprozent, Mn: 0,10 bis 2,0 Massenprozent, P: 0,0250 Massenprozent oder weniger, S: 0,010 Massenprozent oder weniger, Al: 0,0050 bis 0,10 Massenprozent, Sb: 0,010 bis 0,50 Massenprozent, N: 0,0010 bis 0,0080 Massenprozent besteht und ferner zumindest eines ausgewählt aus Cu: 0,010 bis 1,0 Massenprozent und Ni: 0,010 bis 1,0 Massenprozent aufweist und ferner optional zumindest eines ausgewählt aus Cr: 0,050 Massenprozent oder weniger, W: 0,005 bis 0,5 Massenprozent, Mo: 0,005 bis 0,5 Massenprozent, Ti: 0,0010 bis 0,030 Massenprozent, Nb: 0,0010 bis 0,030 Massenprozent, Zr: 0,0010 bis 0,030 Massenprozent, V: 0,0020 bis 0,20 Massenprozent, Ca: 0,0005 bis 0,0040 Massenprozent, REM: 0,0001 bis 0,0150 Massenprozent, Y: 0,0001 bis 0,10 Massenprozent, Se: 0,0005 bis 0,50 Massenprozent, Te: 0,0005 bis 0,50 Massenprozent und Co: 0,010 bis 0,50 Massenprozent aufweist und zusätzlich der Rest Eisen und unvermeidbare Verunreinigen ist.

2. Korrosionsbeständiger Stahl für einen Kohletransporter oder Erz-/Kohle-Transporteraufnahme nach Anspruch 1, wobei
in dem Stahl Cr etwa 0,050 Massenprozent oder weniger beträgt.

3. Korrosionsbeständiger Stahl für einen Kohletransporter oder Erz-/Kohle-Transporteraufnahme nach Anspruch 1 oder Anspruch 2, der
mindestens eines ausgewählt aus W: 0,005 bis 0,5 Massenprozent und Mo: 0,005 bis 0,5 Massenprozent zusätzlich zu dem Stahl aufweist.

4. Korrosionsbeständiger Stahl für einen Kohletransporter oder Erz-/Kohle-Transporteraufnahme nach einem der Ansprüche 1 bis 3, der
zumindest eines ausgewählt aus Ti: 0,0010 bis 0,030 Massenprozent, Nb: 0,0010 bis 0,030 Massenprozent, Zr: 0,0010 bis 0,030 Massenprozent und V: 0,0020 bis 0,20 Massenprozent zusätzlich zu dem Stahl aufweist.

5. Korrosionsbeständiger Stahl für einen Kohletransporter oder Erz-/Kohle-Transporteraufnahme nach einem der Ansprüche 1 bis 4, der
zusätzlich zu dem Stahl Ca: 0,0005 bis 0,0040 Massenprozent aufweist.

6. Korrosionsbeständiger Stahl für einen Kohletransporter oder Erz-/Kohle-Transporteraufnahme nach einem der Ansprüche 1 bis 5, der
zumindestens einen ausgewählt aus REM: 0,0001 bis 0,0150 Massenprozent und Y: 0,0001 bis 0,10 Massenprozent zusätzlich zu dem Stahl aufweist.

7. Korrosionsbeständiger Stahl für einen Kohletransporter oder Erz-/Kohle-Transporteraufnahme nach einem der Ansprüche 1 bis 6, der
zumindestens eines ausgewählt aus Se: 0,0005 bis 0,50 Massenprozent, Te: 0,0005 bis 0,50 Massenprozent und Co: 0,010 bis 0,50 Massenprozent zusätzlich zu dem Stahl aufweist.

## Revendications

1. Acier résistant à la corrosion pour une cale de transporteur de charbon ou de transporteur de minerai / charbon, dans lequel la composition chimique de l'acier consiste en C : 0,010 à 0,200 pour cent en masse, Si : 0,05 à 0,50 pour cent en masse, Mn : 0,10 à 2,0 pour cent en masse, P : 0,0250 pour cent en masse ou moins, S : 0,010 pour cent en masse ou moins, Al : 0,0050 à 0,10 pour cent en masse, Sb : 0,010 à 0,50 pour cent en masse, N : 0,0010 à 0,0080 pour cent en masse, et comprend en outre au moins un élément sélectionné parmi Cu : 0,010 à 1,0 pour cent en masse et Ni : 0,010 à 1,0 pour cent en masse, et comprend en outre de manière facultative au moins un élément sélectionné parmi Cr : 0,050 pour cent en masse ou moins, W : 0,005 à 0,5 pour cent en masse, Mo : 0,005 à 0,5 pour cent en masse, Ti : 0,0010 à 0,030 pour cent en masse, Nb : 0,0010 à 0,030 pour cent en masse, Zr : 0,0010 à 0,030 pour cent en masse, V : 0,0020 à 0,20 pour cent en masse, Ca : 0,0005 à 0,0040 pour cent en masse, REM : 0,0001 à 0,0150 pour cent en masse, Y : 0,0001 à 0,10 pour cent en masse, Se : 0,0005 à 0,50 pour cent en masse, Te : 0,0005 à 0,50 pour cent en masse, et Co : 0,010 à 0,50 pour cent en masse, et de plus, le reste étant du Fe et des impuretés inévitables.

2. Acier résistant à la corrosion pour une cale de transporteur de charbon ou de transporteur de minerai / charbon, selon la revendication 1, dans lequel dans l'acier, Cr est à 0,050 pour cent en masse ou moins.

3. Acier résistant à la corrosion pour une cale de transporteur de charbon ou de transporteur de minerai / charbon, selon la revendication 1 ou la revendication 2, comprenant au moins un élément sélectionné parmi W : 0,005 à 0,5 pour cent en masse et Mo : 0,005 à 0,5 pour cent en masse en plus de l'acier.

4. Acier résistant à la corrosion pour une cale de transporteur de charbon ou de transporteur de minerai / charbon, selon l'une quelconque des revendications 1 à 3, comprenant au moins un élément sélectionné parmi Ti : 0,0010 à 0,030 pour cent en masse, Nb : 0,0010 à 0,030 pour cent en masse, Zr : 0,0010 à 0,030 pour cent en masse et V : 0,0020 à 0,20 pour cent en masse en plus de l'acier.

5. Acier résistant à la corrosion pour une cale de transporteur de charbon ou de transporteur de minerai / charbon, selon l'une quelconque des revendications 1 à 4, comprenant du Ca : 0,0005 à 0,0040 pour cent en masse en plus de l'acier.

6. Acier résistant à la corrosion pour une cale de transporteur de charbon ou de transporteur de minerai / charbon, selon l'une quelconque des revendications 1 à 5, comprenant au moins un élément sélectionné parmi REM : 0,0001 à 0,0150 pour cent en masse et Y : 0,0001 à 0,10 pour cent en masse en plus de l'acier.

7. Acier résistant à la corrosion pour une cale de transporteur de charbon ou de transporteur de minerai / charbon, selon l'une quelconque des revendications 1 à 6, comprenant au moins un élément sélectionné parmi Se : 0,0005 à 0,50 pour cent en masse, Te : 0,0005 à 0,50 pour cent en masse et Co : 0,010 à 0,50 pour cent en masse en plus de l'acier.
